

# United States Patent

[11] 3,615,492

[72] Inventors **Fritz-Walter Lange;**  
Jens E. Muller, both of Gauting, Germany  
[21] Appl. No. **731,730**  
[22] Filed **May 24, 1968**  
[45] Patented **Oct. 26, 1971**  
[73] Assignee **Hans Schwarzkopf G.m.b.H.**  
**Hamburg, Germany**  
[32] Priority **June 1, 1967**  
[33] **Germany**  
[31] **P 15 47 660.5**

[56] **References Cited**  
UNITED STATES PATENTS  
2,875,050 2/1959 Goldberg et al. .... 96/66.3  
FOREIGN PATENTS  
494,468 10/1938 Great Britain..... 96/52  
*Primary Examiner—Norman G. Torchin*  
*Assistant Examiner—Mary F. Kelley*  
*Attorney—Fleit, Gipple & Jacobson*

[54] **PHOTOGRAPHIC DEVELOPER CONTAINING A  
PYRIDINE DERIVATIVE**  
3 Claims, No Drawings

[52] U.S. Cl. .... **96/52,**  
96/66  
[51] Int. Cl. .... **G03c 7/00,**  
G03c 5/30  
[50] Field of Search. .... **96/52, 66,**  
66.3

**ABSTRACT:** The invention provides a developer solution for simultaneously developing and toning positive photographic prints, the solution containing hydroquinone as the developer and a specified pyridine derivative as toning agent to provide a brown-tinted (e.g. yellowish-brown, olive-brown, reddish-brown, or neutral-brown) print.

## PHOTOGRAPHIC DEVELOPER CONTAINING A PYRIDINE DERIVATIVE

This invention relates to photographic developers for obtaining color-toned prints.

It has long been known to tone positive prints by sulfur toning, by metal salt toning with, for example, gold, copper or vanadium salts, or by chromogenous development of the print (E. Mutter: Kompendium der Photographie, Vol. III pages 104-113, Verlag für Radio-Foto-Kinotechnik, Berlin-Borsigwalde, 1963).

However, these methods suffer from substantial disadvantages due, on the one hand, to the complexity of the method concerned—a number of additional working operations are required for developing and often further operations for bleaching and toning—, and on the other hand, to the often unsatisfactory quality of the toned print. In particular the toning often has an unfavorable effect on the grain size of the black silver print and brown-tinted images become clay-yellow, especially when using a sulfur toner. Also overexposed and underdeveloped prints tend to become too bright and deadened pictures take on a blackish tone. In addition, with chromogenous developers the solutions are not stable in storage and must therefore be mixed from two separate containers before being used.

It has also been proposed to achieve a brownish coloration of the print by use of very dilute solutions of hydroquinone (Mutter, Vol. III, pages 79 and 80). Using this method, however, from the exposure time is increased by a factor of from 1.5-7 and also extended developer times are necessary. This provides prints with no contrast and in which the brown tone is hardly detectable. In using some of these developers it is proposed that beige-colored papers should be used, in which not the silver print but the whole surface of the paper is colored.

The present invention has for its aim to provide a developer solution which permits development and toning of the positive print in one working operation without extended exposure or developing times, while maintaining as small a grain size and providing toning of the print, particularly in a neutral-brown coloration.

Surprisingly it has been found that these requirements can be met if there is added to an alkaline hydroquinone-type developer solution, optionally containing a superadditive, such as phenidon, a pyridine compound of the formula:



where  $R_1$ ,  $R_2$ ,  $R_3$ , and  $R_4$  each represent a hydrogen atom, a  $C_1-C_4$  alkyl group, or a hydroxyalkyl, aminoalkyl, or alkoxyalkyl group; and  $X$  and  $Y$  each represent a hydrogen atom, a hydroxyl group or a hydroxyalkyl group.

The pyridine compounds used in the developer solutions of the invention are known compounds and can be prepared by known methods, described, for example, in Den Hertog and Jouwersma, Recueil Trav.chim, Netherlands 72, 125 (1953) and also in Wenner and Plati, J. Org. Chemistry 11, 751 (1946).

The following pyridine compounds included in these general formula have proved to be particularly suitable for additives to hydroquinone developer solutions for toning positive silver prints:

2-hydroxyethylamino-5-aminopyridine  
3,4-diaminopyridine  
2-dimethylamino-5-aminopyridine  
2-N-methylamino-5-aminopyridine, or  
2,3-diamino-6-methoxypyridine.

Using these pyridine additives yellowish-brown, olive-brown, reddish-brown or neutral-brown prints can be obtained depending on the particular additive used.

An advantage of the toning agents used in accordance with the present invention is the fact that they can be added directly to the developer solution, e.g. of the hydroquinone/Metol type, and that development and toning can be achieved in one working operation. Known superadditives, e.g. 1-phenyl-pyrazolone or 1-phenyl-3-amino pyrazolone, can also be added to the developer solution, if desired.

A further advantage of the toning agents used in accordance with the invention lies in the fact that the grain size of the silver print is not unfavorably influenced.

Finally, a further advantage lies in the fact that the exposure and also the developing times do not need to be extended.

The novel toning developers of the invention can be used for all silver halide papers, the tone effect being clearer on silver chloride paper than on silver bromide paper.

The intensity of the desired tone effect can be adjusted precisely with the concentration of the pyridine compound in the developer solution. Very weak tone effects can be achieved with a concentration of 0.01 percent of toning agent while a concentration of 1.0 percent gives extremely strong tone effects. The pyridine compounds should preferably be present in the developer solution in an amount of from 0.05 to 0.3 percent. The concentration of developer and super additive, if any, is entirely conventional.

The following examples illustrate developer solutions in accordance with the invention.

## EXAMPLE 1

A toning developer was made up according to the following formulation:

|              |                                     |
|--------------|-------------------------------------|
| 1.5 g.       | sodium sulfite,                     |
| 2.3 g.       | sodium carbonate,                   |
| 0.06g.       | potassium bromide,                  |
| 0.4 g.       | hydroquinone,                       |
| 0.02 g.      | phenidon                            |
| 0.1 g.       | 2-hydroxyethylamino-5-aminopyridine |
| q.s. 100 ml. | distilled water                     |

Using this developer solution silver chloride paper which had been exposed for 20 seconds with a neutral wedge filer, was developed for 1½ minutes, fixed and then washed. A neutral-brown-toned silver print was obtained.

In a comparative experiment, the pyridine derivative was replaced by 0.1 g. of Metol. A silver chloride paper exposed and developed therein under the same conditions as previously gave an untoned neutral-black silver print.

## EXAMPLE 2

A developer solution was made up as in example 1 but using 0.06 g. of 2-N-methylamino-5-aminopyridine in place of the 2-hydroxyethylamino-5-amino pyridine.

A silver chloride paper exposed and developed therewith produced a clearly reddish-brown-toned silver print.

## EXAMPLE 3

A developer solution was made up as in example 1 but using 0.4 g. of 2,6-dimethoxy-3-aminopyridine as the pyridine additive. A silver chloride paper exposed and developed with this developer gave an olive-brown-toned silver print.

## EXAMPLE 4

A developer solution was made up as follows:

|              |                               |
|--------------|-------------------------------|
| 1.3 g.       | sodium sulfite                |
| 1.9 g.       | sodium carbonate,             |
| 0.04 g.      | potassium bromide,            |
| 0.35 g.      | hydroquinone,                 |
| 0.1 g.       | p-methylaminophenol           |
| 0.1 g.       | 2,3-diamino-6-methoxypyridine |
| q.s. 100 ml. | distilled water               |

Using this developer solution an exposed silver chloride paper was developed as in example 1. The result was a strong neutral-brown-toned silver print.

## EXAMPLE 5

A developer solution was made up as follows:

|              |                     |
|--------------|---------------------|
| 1.5 g.       | sodium sulfite      |
| 2.2 g.       | sodium carbonate    |
| 0.05 g.      | potassium bromide   |
| 0.4 g.       | hydroquinone        |
| 0.1 g.       | p-methylaminophenol |
| 0.02 g.      | phenidon            |
| 0.1 g.       | 3,4-diaminopyridine |
| q.s. 100 ml. | distilled water     |

Using this developer solution an exposed silver bromide paper was developed for 2 minutes, washed and then fixed. A yellowish-brown-toned silver print resulted.

We claim:

1. In an alkaline photographic developer solution containing hydroquinone as the developer the improvement comprising a toning additive in an amount of from 0.01-1.0 percent, said additive being selected from pyridine compounds of the formula

5



wherein: R<sub>1</sub>, R<sub>2</sub>, R<sub>3</sub> and R<sub>4</sub> are each selected from hydrogen, C<sub>1</sub>-C<sub>4</sub> alkyl groups, hydroxyalkyl groups, aminoalkyl groups and alkoxyalkyl groups; and X and Y are each selected from hydrogen, hydroxyl groups and alkoxy groups.

2. An alkaline photographic developer solution as claimed in claim 1, wherein the amount of toning additive is 0.05-0.3 percent.

3. An alkaline photographic developer solution as claimed in claim 1, wherein the toning additive is selected from:

2-hydroxyethylamino-5-aminopyridine  
3,4-diaminopyridine  
2-dimethylamino-5-aminopyridine  
2,6-dimethoxy-3-aminopyridine  
2-N-methylamino-5-aminopyridine, and  
2,3-diamino-6-methoxypyridine.

25

30

35

40

45

50

55

60

65

70

75